

## UNITED STATES PATENT OFFICE

2,200,286

## UNINEGATIVE MULTICOLOR PLANOGRAPHY

Gustave R. Lukesh, Pasadena, Calif., and John G. Goedike, San Antonio, Tex.

o Drawing. Application April 13, 1939,  
Serial No. 267,676

7 Claims. (Cl. 95—5.2)

(Granted under the act of March 3, 1883, as  
amended April 30, 1928; 370 O. G. 757)

This invention described herein may be manufactured and used by or for the Government for governmental purposes, without the payment to us of any royalty thereon.

5 This invention relates to a process of multicolor reproduction from planographic and other analogous printing presses and in the present case is called uninegative multicolor planography, as only one photographic negative is used in the process to obtain several planographic or photolitho process press plates of progressive color value for the reproduction of the original copy in multicolor.

10 This process may be used for the reproduction of any subject or original copy in multicolor and is particularly valuable as a method of reproducing such single hued copy as air pictures, air mosaics, wash drawings and photographic copy in multicolor by the planographic process. It is known that the use of color filters and the circular screen will obtain photographic negatives of distinct color values from any colored copy, but by this process it is possible to supply color values for single hued copy and from one photographic negative.

15 Monochromatic planographic reproduction of any pictorial subject of a single hue will give a very flat result or a result that has lost much of the detail if any contrast is obtained. It is contemplated by this invention to use a single photographic negative of normal exposure and development to obtain several and distinct planographic press plates of progressive color value to be run in colors, varying from a light color such as yellow to a dark blue, and obtain a multi-colored reproduction of the subject. Treatment in this manner will permit the introduction of an increase in the qualities of form and relief; intensification and clarification of features and detail; embellishment; introduction of color contrast, color harmony, and/or color complement as desired.

20 In carrying out the invention, the process consists in producing a single photographic negative of normal exposure and development of a pictorial subject to be reproduced in multicolors. A contact positive may be made of the negative and then a master negative of the same size as a planographic plate may be made of the positive.

25 To produce a multicolor reproduction of the subject from the master negative, a plurality of time controlled exposures of the negative is made upon a plurality of planographic plates which are treated progressively, each plate being

grained to the correct texture for the color intended. The surface of the plate for the lightest color such as yellow receives the finest grain. The surface of the plate or plates for the intermediate colors such as red and the like, receives a grain coarser in texture than the plate for the lightest color and the surface of the plate for the darkest color such as dark blue receives the coarsest grain in the series, whereby progressive light sensitive coatings of varying sensitivity are provided on the plates.

30 In order to aid in obtaining progression in the light sensitive coatings on the plates of the series, suitable light sensitive solutions may be used on the light sensitive coatings with the exposures of the negative to the plates being timed with respect to the sensitivity of the light sensitive solutions. The solutions are selected with respect to the sensitivity of the light sensitive coatings on the plates, and as an example the following formulae may be used to obtain progression in the light sensitive coatings on the plates of the series as above described. It is to be understood, however, that these formulae are given without intending to confine the process to the formulae.

35 To give an extremely light sensitive coating to a plate, the first solution may be composed as follows:

|                     |              |     |    |
|---------------------|--------------|-----|----|
| Water               | fluid ounces | 160 | 30 |
| Egg albumen flakes  | ounces       | 16  |    |
| Ammonium bichromate | do           | 3   |    |
| Aqua ammonia, 28%   | fluid ounces | 3   | 35 |

40 To give a less sensitive coating to a plate which develops easily, the second solution may be composed as follows:

|                      |              |     |    |
|----------------------|--------------|-----|----|
| Water                | fluid ounces | 160 | 40 |
| Photoengravers' glue | do           | 32  |    |
| Ammonium bichromate  | ounces       | 3   |    |
| Aqua ammonia, 28%    | fluid ounces | 3   |    |

45 The plate for the lightest color of the series may be coated in the usual manner with the first solution and in a vacuum frame under the negative it is given extreme exposure to light. All the modeling, in the light tones of the subject, is burned on to this plate and the modeling in the dark shadows is disregarded and will go solid and lose character.

50 The plate for the intermediate color of the series may be coated with a composite solution

which is proportioned of the two solutions given and mixed as follows:

|                        | Fluid ounces |
|------------------------|--------------|
| 1st solution (albumen) | 14           |
| 5 2nd solution (glue)  | 2            |

This intermediate color plate is exposed in the usual manner under the negative in the vacuum frame and the exposure timed to obtain the modeling and detail of the intermediate tones. 10 Much of the detail of the light tones will be lost on this plate and much of the dark tones of the subject will close solid.

The plate for the darkest color such as dark blue of the series is coated with a composite solution proportioned of the two given solutions and mixed as follows:

|                        | Fluid ounces |
|------------------------|--------------|
| 1st solution (albumen) | 12           |
| 20 2nd solution (glue) | 4            |

This plate may be exposed under the negative in the vacuum frame in the usual manner and the exposure to the light timed to obtain the detail in the deep tones of the subject. All the 25 detail in the light tones of the subject are lost from the surface of this plate but some of the intermediate tones will hold.

The plates after exposure to the negative may then be treated for use on a press, such as by 30 coating the plates of the series with developing ink and developing them under water, and after developing flowed with a thin solution of gum arabic which contains a trace of a suitable acid, such as phosphoric, and placed in the whirler to 35 dry with the heat on. Drying in a temperature between 150 to 180 degrees F. seasons the design on the surface of a plate and it becomes resistant enough to stand an acid treatment for fixation.

40 Each plate may then be allowed to cool after drying and heating and then soaked under water for a few minutes to soften the gum coating and rinsed with water, then without being permitted to dry it is flowed with a weak solution of hydro-fluoric acid in water. The action of the hydro-fluoric acid is to eat away all dead or exposed albumen which might tint up on the press.

After treatment with hydrofluoric acid the 50 plate surface could be flowed with a thin desensitizing solution of gum arabic and phosphoric acid and dried in the whirler. The plate is then ready for the press.

Depending on the subject and the color effect desired the number of progressive color plates 55 may be increased from three to as many as may be required. In making a three color separation from one negative the light color plate of the series will register detail from the lightest tones to a point between the quarter and half tones, 60 the intermediate color plate will register detail from a point between the quarters and half tones to a point between the half and three quarter tones and the dark color plate of the series will register detail from a point between the half and 65 three quarter tones to the full tone.

The developed light sensitive surfaces of the plates are coated with inks of varying color selected with respect to the sensitivity of the corresponding light sensitive surface, thereby providing a plurality of separate and distinct planographic press plates of progressive color value to be run in colors varying from a light yellow to a dark blue, which may be impressed on a 70 printing surface in proper sequence to supply 75

tone effects of primary, secondary and tertiary colors to the reproduced subject.

The process above described is based partly on the discovery that a light sensitive coating for metal planographic press plates may be governed so that the light sensitive properties can be varied from high to low contrast as desired. This effect of degree of contrast is common to sensitive photographic plates and film, but it is new to take advantage of the sensitive degree 10 of the coating on metal planographic plates for the purpose of color separation. The process is further based on the discovery that (with or without such control of light sensitive coating), by controlling the number of plates, by selecting the 15 appropriate grain for each plate, by controlling the exposure of the light-sensitive coatings to light, by selecting appropriate colors and tones of inks and developing the exposures, a result of 20 color separation and/or color superimposition is achieved, producing a print in selected and controlled colors, all from a single original negative, without recourse to color filters.

The use of one negative for making the progressive color plates precludes the possibility of 25 distortion, as each plate will register perfectly to the other plates of the series.

As many progressive color plates may be used as the subject and the desired color effect require. The color scheme will govern the color of 30 the impression for each plate of the series.

It will thus be seen there is provided a highly useful and efficient process for the reproduction in multicolors of an original copy from a single photographic negative. Even though there have 35 herein been described certain steps in carrying out the process, it is nevertheless to be understood that various changes may be made therein without departing from the spirit or scope of the invention.

Having described our invention, what we claim as new and wish to secure by Letters Patent is:

1. A process for making a multicolor reproduction from a single monochromatic original which consists in making a plurality of variably timed 45 exposures of said original upon a succession of light sensitive surfaces, each surface having a different sensitivity than the others thereof, varying from a slight sensitivity to an extreme sensitivity, the sensitivity of the surfaces being related 50 to the colors intended and the timing of the exposures of said original upon said light sensitive surfaces being directly related to the sensitivity of said surfaces, developing said exposed light sensitive surfaces to form a plurality of printing 55 surfaces, coating said developed light sensitive surfaces with inks of variable color selected with respect to the sensitivity of said surfaces and with respect to the timing of the exposures of said original upon said light sensitive surfaces 60 and successively impressing each of said coated surfaces in proper sequence upon a receiving surface.

2. A process for making a multicolor reproduction from a single monochromatic original which 65 comprises making a plurality of variably timed exposures of said original upon a succession of light sensitive surfaces of variable color sensitivity, each surface having a different color sensitivity than the others thereof, varying from a 70 slight color sensitivity to an extreme color sensitivity, the sensitivity of the surfaces being related to the colors intended, and the timing of the exposures of said original upon said light sensitive surfaces being directly related to the color 75

sensitivity of said surfaces, developing said exposed light surfaces to form a plurality of printing surfaces, coating said developed light sensitive surfaces with inks of variable color selected with respect to the sensitivity of said surfaces and with respect to the timing of the exposures of said original upon said light sensitive surfaces and successively impressing each of said coated surfaces in proper sequence upon a receiving surface.

3. A process for making a multicolor reproduction from a single monochromatic original which comprises making a plurality of variably timed exposures of said original upon a succession of light sensitive surfaces of variable sensitivity, varying from a slight sensitivity to an extreme sensitivity, each of said surfaces being differently grained from the others thereof varying from a fine grain to a coarse grain, the colors being selected with respect to the graining of said plates, the sensitivity of said surfaces being related to the graining thereof and the timing of the exposures of said original upon said light sensitive surfaces being directly related to the graining of said surfaces, developing said exposed light sensitive surfaces to form a plurality of printing surfaces, coating said developed light sensitive surfaces with inks of variable color selected with respect to the graining of said light sensitive surfaces and with respect to the timing of the exposures of said original upon said light sensitive surfaces and successively impressing each of said coated surfaces in proper sequence upon a receiving surface.

35 4. A process for making a multicolor reproduction from a single monochromatic original which comprises making a plurality of variably timed exposures of said original upon a succession of planographic plates having light sensitive surfaces of variable sensitivity, each surface of said plates having a different sensitivity than the others thereof varying from a slight sensitivity to an extreme sensitivity, the sensitivity of the surfaces being related to the colors intended and the timing of the exposures of said original upon said light sensitive surfaces of said plates being directly related to the sensitivity of said surfaces, developing said exposed light sensitive surfaces on said plates to form a plurality of printing surfaces, coating said exposed light sensitive surfaces of said plates with inks of variable color selected with respect to the sensitivity of said surfaces and the timing of the exposures of said original upon said light sensitive surfaces, and successively impressing each of said coated surfaces of said plates in proper sequence upon a receiving surface.

5. A process for making a multicolor reproduction from a single monochromatic original which comprises making a plurality of variably timed exposures of said original upon a series of planographic plates, each plate being differently grained from the others thereof varying from a fine grain to a coarse grain, whereby progressive depth of light sensitive coatings is provided on the plates, the sensitivity of said light sensitive coatings on said plates being related to the graining of said plates and the colors intended and the timing of the exposures of said original upon said light sensitive coatings of said plates being directly related to the sensitivity of said coatings, developing said exposed light sensitive coatings of said plates to form a plurality of printing surfaces, coating said developed light sensitive coatings with inks of variable color selected with respect to the sensitivity of the light sensitive coatings and with respect to the timing of the exposures of said negative upon said light sensitive coatings and successively impressing each of said inked light sensitive coatings in proper sequence upon a receiving surface.

ings of said plates with inks of variable color selected with respect to the sensitivity of the light sensitive coatings and with respect to the timing of the exposures of said original upon said light sensitive coatings and successively impressing each of said light sensitive coatings of said plates in proper sequence upon a receiving surface.

6. A process for making a multicolor reproduction of a subject from a single photographic negative which comprises graining a series of planographic plates to obtain progressive depth of light sensitive coatings on the plates, each plate having been differently grained from the others thereof varying from a fine grain to a coarse grain, coating the light sensitive coatings of said plates with light sensitive solutions of variable sensitivity selected with respect to the sensitivity of the light sensitive coatings on the plates, whereby light sensitive surfaces are provided on the plates of variable sensitivity, making a plurality of variably timed exposures of said negative in succession upon the light sensitive surfaces on said plates, the graining of said plates being related to the sensitivity of said plates and the colors intended and the timing of the exposures of said negatives upon said light sensitive surfaces being directly related to the sensitivity of said surfaces, developing said light sensitive surfaces to form a plurality of printing surfaces, coating said developing light sensitive surfaces with inks of variable color selected with respect to the graining of said plates and sensitivity of said surfaces and with respect to the timing of the exposures of said negative upon said light sensitive surfaces and successively impressing each of said coated surfaces of said plates in proper sequence upon a receiving surface.

7. A process for making a multicolor reproduction from a single photographic negative which comprises progressively graining a series of metal planographic plates to the correct texture of the color intended, varying from a fine grain to a very coarse grain, thereby obtaining progressive depth of light sensitive coatings of variable sensitivity on said plates, the sensitivity of the light sensitive coatings being related to the graining of said plates and the colors intended, the finer the grain of said plates the lighter the colors intended, making a plurality of variably timed exposures of said negative in succession upon the light sensitive coatings of said plates, controlling the timing of the exposures to light of said negative upon the light sensitive coatings of said plates, the finer the grain of said plates the more the time interval of exposure of said negative to the light sensitive coatings on said plates, the timing of the exposures of said negative on said light sensitive coatings of said plates being directly related to the sensitivity of said coatings, developing said light sensitive coatings on said plates to form a plurality of printing surfaces, coating said developed light sensitive coatings with inks of variable color selected with respect to the sensitivity of the light sensitive coatings and with respect to the timing of the exposures of said negative upon said light sensitive coatings and successively impressing each of said inked light sensitive coatings in proper sequence upon a receiving surface.

GUSTAVE R. LUKESH.  
JOHN G. GOEDIKE.